

Feb. 17, 1959

P. ROBINSON  
FERRO MAGNETIC CORE MATERIALS AND  
METHODS OF PRODUCING SAME  
Filed Oct. 13, 1955

2,873,512

FIG. 1



FIG. 2



INVENTOR.  
PRESTON ROBINSON

BY  
*Cinnally and Gandy*  
HIS ATTORNEYS

1

2,873,512

## FERRO MAGNETIC CORE MATERIALS AND METHODS OF PRODUCING SAME

Preston Robinson, Williamstown, Mass., assignor to Sprague Electric Company, North Adams, Mass., a corporation of Massachusetts

Application October 13, 1955, Serial No. 540,238

6 Claims. (Cl. 29—182.5)

The present invention relates to magnetic circuit components such as cores and to methods of producing the same.

Because of various design considerations known to electrical engineers, magnetic cores for electrical applications should have high permeability and magnetic saturation together with low electrical losses. The so-called laminated cores consisting of various layers of ferro-magnetic material have been developed to satisfy these requirements. They possess the required permeability and magnetic saturation, but unfortunately the electrical losses with these laminated cores are somewhat higher than are desired for most applications.

Another type of core which has been developed is the so-called powder or dust core consisting of a ferro-magnetic powder or dust pressed and sintered into the desired shape. These cores have very low losses, but because of their inherent structure, do not possess as high a permeability and magnetic saturation as the laminated cores indicated above.

It is an object of the present invention to produce magnetic circuit components which have the high permeability and saturation of the so-called laminated cores, and which also possess low electrical losses as in the dust cores. The second object of the invention is to develop various procedures for producing these circuit components. These and further objects of the invention will be apparent from the following description of several of its exemplifications, reference being made to the accompanying drawings wherein:

Fig. 1 is a fragmentary view of a magnetic core embodying the present invention; and

Fig. 2 is a plan view of a different form of magnetic circuit component illustrative of the present invention.

According to the present invention, individual magnetic metallic elements are provided with an adherent magnetic ferrite coating, and are then assembled into compact form. If desired, the so produced form may be subjected to a sintering operation to render it more coherent.

The base materials for the individual coated particles of the present invention preferably are of "soft" magnetic iron or iron alloys such as iron silicon alloys containing up to 6% of silicon, iron-nickel alloys such as that containing by weight 77.2% nickel, 4.8% copper, 1.5% chromium, the balance being iron. It is to be understood that the present invention is not to be limited to these specific materials but can be employed with substantially pure iron and other iron alloys which are "hard" magnetic compositions. The latter materials can be used to advantage in the production of permanent magnetic compositions. Most of these materials are listed in Appendix 4 of Bozorth's "Ferromagnetism," New York, Van Nostrand, 1951.

The thickness of the uncoated metal elements is of substantial importance and depends upon the final properties desired in the finished material. The base metal

2

can be varied in thickness up to about 40 mils, but is it preferred for high frequency operation to limit the size to as small as convenient, i. e. between about 4 microns and about 25 microns. The metal elements can be either

5 finely divided particles, or thin sheets or wires. Where particles are used, they can be of mixed sizes or of substantially the same diameter and roughly may be taken as corresponding to the fraction retained upon any one screen of the Tyler series. The term "diameter" as used herein is to be taken loosely as the invention is not limited to precise spheres but is applicable to odd shaped pieces of metal.

A feature of the present invention is that the magnetic ferrite coatings not only electrically insulate the metallic elements from each other, but, by reason of their good magnetic characteristics, do not act as air gaps that otherwise seriously dilute the metallic particles. In other words, by means of the present invention, the metallic particles are so well insulated from each other that eddy current losses are sharply reduced, yet at the same time the assembly of insulated elements is essentially entirely composed of magnetic material.

Suitable magnetic ferrites for use in accordance with the present invention are the so-called mixed crystal ferrites such as those described in the Snoek et al. U. S. Patents Nos. 2,551,711, 2,579,978, 2,636,860, and Crowley U. S. Patent No. 2,575,099. Simple ferrites such as those described in U. S. Patent No. 1,946,964 can also be used.

15 30 The adherent ferrite coatings of the present invention are formed by providing the surface of the base with a suitable precoating and then heat treating the so precoated material at temperatures of from 900° C. to 1400° C. for periods of from 2 to 5 hours in length.

35 40 This treatment may be carried out in a number of gases such as technical nitrogen, oxygen or air. For some ferrites such as a manganese ferrite, it is advantageous to employ an oxygen-poor atmosphere in order to hold the stoichiometric proportions of oxygen in the final material so as to correspond to the desired valence of manganese.

When a homogeneous mixed crystal ferrite is used with the present invention, the choice of which mixed

45 crystal system to employ varies with the individual design considerations involved. Frequently, it is desirable to have as high an initial permeability of the ferrite coating as possible. This can be provided by selecting a composition having a low Curie temperature, but the Curie temperature should not be in the range of temperatures at which the magnetic component is to be operated.

50 55 A very effective technique for applying the ferrite coatings is by means of a fluidized bed such as used in the petroleum industry. Because of the nature of the

55 materials employed, it is preferred to use a fixed bed with this invention but moving beds can also be employed. With fixed beds, the velocity of the individual gases employed to suspend the particles is normally chosen so that the bed is in continuous quiescent agitation.

60 With particles of from 40-50 microns in diameter, velocities from 0.01 feet per second to about 0.1 feet per second accomplish this end. With particles in the preferred diameter range noted above, the velocities should be in the order of about 1.5 feet per second.

65 70 Higher velocities than this may be used, however, but when they are used, slug flow is apt to result and the individual particles will not be uniformly treated. When velocities are too low the desired agitation is not obtained. Inasmuch as the conditions for fluidized treatment have been well worked out and are available in the art they will not be further elaborated here.

The initial suspension of the metallic particles in a

fluidized bed may be accomplished with any one of a number of gases, such as hydrogen, oxygen, nitrogen, or air. It is preferred, however, to initially use gases which will not oxidize the individual particles, such as nitrogen, and to utilize these gases to heat the bed to a temperature of around 500 to 1,000° C. This can, of course, be accomplished by the use of gas temperatures of approximately this same range. Additional heating means, such as jackets, induction coils, and the like can be employed throughout the various steps herein specified.

After the bed of particles has been brought to an appropriate temperature, the external surfaces of the individual metal pieces are oxidized in accordance with this invention by treatment with an oxidizing gas, such as oxygen or air for a period of between 10 seconds and five hours depending upon the reaction conditions employed and the final coating thickness desired. It is best to run several tests to determine the precise degree of oxidation and temperatures for use with any given type of particle. Certain alloys contain substituents, such as aluminum, which tend to form undesirable impervious films upon oxidation. The use of large amounts of these film forming metals is, in general, to be avoided.

Occasionally, it is desirable to combine the particle heating step and the oxidizing treatment into a single operation in which either air or oxygen or the like is used to both heat and oxidize the metallic bases employed. Because such a combined operation is difficult to control, it is normally preferable to avoid it.

After the oxidation in the fluidized bed has been completed, one or more additional oxides of the type needed to make the desired ferrite is deposited upon the individual particles as by the thermal decomposition of an appropriate metal alkoxide, as described in the copending Robinson application, Serial No. 311,529, filed September 25, 1952. Suitable alkoxides are zinc methoxide, magnesium ethoxide, copper (ous) propoxide, and the like. Other components capable of yielding a metallic oxide besides those listed can, of course, be employed, but the alkoxides are preferred because of their volatility and ease of decomposition under the reaction conditions involved. Frequently, it is desirable to aid the passage of these gases through a fluidized bed by the use of from 10% to 95% of a non-reactive carrier gas such as nitrogen.

The individual gases employed during this step of the process should preferably be heated to immediately below their decomposition points in order to facilitate the production of the final coating. Occasionally, it is necessary to stop the deposition of oxides before the desired amount of these components have been deposited and re-heat the metallic bases used in order that the thermal decomposition may proceed at a satisfactorily rapid rate.

After the desired oxide coatings have been deposited, the particles are heated at from 900 to 1400° C. for a period of one-half to five hours in length as indicated above in order to convert the mixed oxides to the ultimate ferrite.

Since the ferrites as formed above are sometimes adversely affected by rapid cooling, it is desirable to slowly cool the hot particles at a rate of about 10 to 100° C. per minute. The cooling can be carried out either by a fluidized bed technique or in any other desired manner.

The thickness of the ferrite coatings can vary widely depending upon the final properties desired. In general, they should not be so thin that they are apt to be damaged during subsequent treatment. However, thin coatings are generally the most adherent. A one mil thickness is about the maximum that is suitable, and in general thinner coatings, from 5 to 15 microns thick, for example, are preferred.

Referring now to the drawings, Fig. 1 shows in enlarged view one form of magnetic circuit component construction made from base elements in the form of finely divided particles or powder. The base elements are represented at 10, each element carrying an adherent sur-

face coating 12 of magnetic ferrite. Where the coated particles are sintered together, the coatings on adjacent particles run together and become integral. Such a particulate construction can, by suitable shaping and molding, be used to make magnetic cores, shells, toroids or the like.

In Fig. 2 there is shown a toroid-type loop core made of strip or foil 16 spirally wound. The individual turns of the winding are insulated from each other by an adherent magnetic ferrite coating 18 which can be applied to one or both faces of the strip. After the coated strip is wound up, it can be subjected to a sintering operation to cause coatings on adjacent faces to cohere together and help bond the turns in the desired shape. The strip thickness should not be greater than the dimensions indicated above for the particles of Fig. 1. In general, however, the strip should be as thin as practical since the eddy current losses for a strip are usually somewhat higher than for the powder type construction.

Instead of having the strip wound as a continuous spiral, it can be cut into individual lengths which can be laminated together in the usual type of core construction. Alternatively a continuous spiral as in Fig. 2 can be cut into two pieces so as to simplify the application of windings to carry the electric currents, when the magnetic component is used as part of an inductor. The cut pieces can be joined together after the windings are applied. Although only about three turns of winding are shown in Fig. 2, this is only in the interest of simplicity and any number of turns can be used.

The following examples of the invention are given for purposes of illustration only and are not to be considered as limiting the invention in any manner.

#### Example I

A 1/2" internal diameter tube 30" high is placed over a supporting manifold consisting of a gas inlet chamber, a compact gas distributing section and a 20 mesh supporting screen. 20 lbs. of silicon-iron alloy particles containing 4% silicon and 96% iron having an average particle diameter of about 0.0224" is placed within the tube above the supporting screen. Heated nitrogen at about 1400° C. is then admitted to the bottom of the column so that it passes through it at a velocity of about 0.837 ft. per second. This velocity is maintained for all gas flow through the fluidized treatment. At this velocity each individual particle is surrounded by a thin film of gas and is subjected to a slight amount of agitation. After a period of 15 minutes, technical oxygen at 700° C. is passed through the bed for a period of 1 minute. Manganese ethoxide is then passed through the bed along with 80% nitrogen at about 900° C. for a period of 10 minutes. At the end of this time zinc methoxide is passed through the bed along with 80% nitrogen for a period of 15 minutes. The particles are then brought up to the 1400° C. temperature by passing heated nitrogen through the bed as before for a period of 15 minutes. Following this the bed is gradually cooled at a rate of 50° C. per minute by the passage of progressively cooling nitrogen through the bed.

#### Example II

Coated particles are formed using the same apparatus, reactants, and conditions specified in Example I except for the following changes:

- 65 (1) Nickel propoxide is used instead of manganese ethoxide.
- (2) The final heating is at a temperature of 1250° C. for a period of 4 hours.

In some cases it is possible to incorporate the metallic ingredients of either a single or a mixed crystal ferrite within the base material, and form the product by oxidation without a pre-coating step. By way of example, the base can be an alloy of iron and nickel, or iron nickel and manganese, or it can be iron having thin platings of the above metals.

*Example III*

Five pounds of particles consisting of the stoichiometric metal composition of a cobalt ferrite and having an average diameter of 0.0224 inch are placed within the apparatus of Example I. Air at 600° C. is passed through the particle bed for a period of five minutes at a velocity of 0.915 ft./sec.; then 1300° C. nitrogen is passed through it at substantially the same velocity for a period of three hours; finally, the particles are cooled to room temperature by decreasing the nitrogen temperature at the rate of 20° C./min.

Frequently the initial iron or iron alloys employed with the invention contain impurities such as carbon and sulfur which have undesirable effects upon the magnetic properties of the final product. These impurities can often be removed to a large extent by initial treatment with hydrogen, as indicated in the following example:

*Example IV*

Coated particles are produced as in Example I except for the passage of hydrogen at 1000° C. through the bed for a period of 30 minutes immediately before the oxidizing treatment.

The formation of individual circuit elements such as cores from the particles produced in accordance with the preceding discussion in effect follows the broad procedures known to the art. The particles are placed in a mold and subjected to pressures of from 10 lbs. per square inch to approximately 100 tons per sq. inch, removed from them old, and if desired, sintered. On many occasions it is advantageous to employ from 1 to 5% of a binding agent such as gum tragacanth, polyvinyl alcohol, dextrin, gum arabic, or the like, to hold the individual particles together during the pressing of the core and immediately thereafter. The use of these binding materials does not have a disadvantageous effect and they can be removed from the core material as by heating to temperatures at which they burn off or are volatilized.

A final sintering of the pressed cores is quite desirable. Not only does it help reduce the air gaps in the pressed material, but if carried out at temperatures of from 900 to 1400° C. and the resulting product is properly cooled as indicated above, the permeability of the ferrite coating usually becomes noticeably higher. Of course, it will be realized that the sintering step serves to more securely bond the individual particles together if carried out for a sufficient length of time, as for example from 1 to 4 hours.

*Example V*

Particles produced in accordance with the procedure of Example I are placed in a mold one inch in diameter and 6 inches long and subjected to a pressure of 25 tons per square inch. The pressure is then relieved and the pressed mass removed from the mold.

*Example VI*

The core produced in Example V is next sintered at 1200° C. in a nitrogen atmosphere for a period of 3 hours, and cooled in the same atmosphere at a rate of 50° C. per minute until a temperature of 25° C. is reached.

*Example VII*

Particles coated as indicated in Example I are mixed with 2% polyvinyl alcohol in a tumbling drum, and then are treated in accordance with the procedures of Examples V and VI.

When permanent magnetic cores are described, it is advantageous to subject "hard" ferro-magnetic coated particles to a magnetic field of from 1000 to 10,000 oersteds while cooling them from above the Curie points of all of the substituents involved. This may be quite easily accomplished immediately after the sintering. By this expedient, permanent magnets are obtained which have the advantageous properties of the power magnets such as have been produced by Dean and Davis, U. S. Patent

No. 2,239,144, and which are stable, i. e. not easily corroded or oxidized in an oxidizing atmosphere.

*Example VIII*

During the cooling of a core sintered as indicated in the preceding Example VI a transverse field of 5,000 oersteds is applied to the core until a temperature of 25° C. is reached.

*Example IX*

10 An 0.25 mil thick strip of  $\frac{1}{4}$  wide transformer iron containing 1% silicon is unreeled and passed continuously through an oven in which it is heated to 800° C. in the presence of air for 4 minutes. The strip is then moved through another oven where it is heated to 400° C. and exposed to the vapors of magnesium ethoxide for 8 minutes. The strip is then subjected to a third similar treatment at 400° C. in an atmosphere of zinc ethoxide for 3 minutes. The strip is exposed in all treatments so that both faces become coated in each oven. The strip is then passed through a fourth oven where it is heated to 1100° C. for 30 minutes, and then cooled to room temperature at a rate of 10° C. per minute. The resulting material makes a very effective core when merely wound up in spiral form. It is further improved by taking the wound core and reheating it at 1400° C. for 30 minutes in an oxygen-free atmosphere. This reheating causes the coatings to sinter together and the spiral will then be a coherent body that is more readily handled.

20 The above Example IX can be modified by omitting the zinc ethoxide treatment, or by substituting for this treatment a corresponding treatment with manganese methoxide.

25 Instead of having the iron oxide coating formed by heating in air or oven, it can be formed in other ways as by anodically treating the iron or iron alloy base material in an electrolyte such as ammonia or dilute sodium hydroxide, which does not dissolve iron oxide. The anodic current density should be relatively low, as for example less than 10 amperes per square foot, in order to form the oxide at a relatively slow rate so that it adheres to the anode and does not flake off. The other oxides can also be deposited in other manners, as for example by applying to the base material a finely divided form of oxide such as magnesium oxide suspended in a medium such as 30 a dilute solution of cellulose nitrate or other resin in an appropriate solvent. Such oxide coatings are, however, more friable and should be subjected to only very gentle handling until after they are fired and converted to ferrite. Such conversion causes the more or less friable oxide layer to become bonded to the iron oxide layer underneath it.

35 The ferrite coatings of the present invention can also be deposited on non-magnetic bases. For example, magnesium-manganese ferrites such as those containing manganese in amounts corresponding to about 15%  $Mn_3O_4$  make good rectangular hysteresis bodies.

40 These ferrites can be deposited in a layer up to about 5 mils thick on ceramic forms such as rings having an internal diameter of 50 mils, an external diameter of 70 mils and 30 mils thick. All the ferrite ingredients can be deposited by thermal deposition or by oxidation of metal coatings or partly one way and partly another. In general, the ferrites should have approximately stoichiometric composition.

45 As many apparently widely different embodiments of this invention may be made without departing from the spirit and scope hereof, it is to be understood that the invention is not limited to the specific embodiments set forth except as defined in the appended claims.

50 This application is a continuation-in-part of application Serial No. 310,719, filed September 20, 1952.

55 What is claimed is:

1. A magnetic circuit component comprising an assembly of thin ferromagnetic metal individual finely divided particles less than about 40 mils thick, the elements

being electrically insulated from each other by surface coatings less than 1 mil thick of magnetic ferrites.

2. The combination of claim 1 in which the coated particles are sintered together, the coatings on adjacent particles being integral.

3. A ferro-magnetic electrical core consisting of individual magnetic iron finely divided particles less than about 40 mils thick provided with magnetic ferrite coatings less than 1 mil thick.

4. A process of preparing a magnetic circuit component, which process includes the steps of providing ferro-magnetic metal individual finely divided particles less than 40 mils thick with surface coatings of magnetic ferrites less than 1 mil thick, and sintering and running together coatings on adjacent particles to form an integral particle coating and hold the particles together in an assembly of such elements to form a coherent body.

5. The combination of claim 1 in which the thin metal elements are between 4 and 25 microns in thickness, and their surface coatings are between 5 and 15 microns thick.

6. The combination of claim 1 in which the thin metal elements are contiguous portions of an elongated metal strip wound up in the form of a loop.

References Cited in the file of this patent

UNITED STATES PATENTS

|    |           |              |               |
|----|-----------|--------------|---------------|
| 10 | 2,068,658 | Cox          | Jan. 26, 1937 |
|    | 2,179,810 | Brill        | Nov. 14, 1939 |
|    | 2,365,720 | Neighbors    | Dec. 26, 1944 |
|    | 2,418,467 | Ellis et al. | Apr. 8, 1947  |
| 15 | 2,563,520 | Faus         | Aug. 7, 1951  |
|    | 2,783,207 | Tombs        | Feb. 26, 1957 |